

Patented Aug. 28, 1928.

1,682,561

# UNITED STATES PATENT OFFICE.

EARL C. HENNEN, OF CHARLESTON, WEST VIRGINIA, ASSIGNOR TO THE UNITED STATES NITO CO., INC., OF COLUMBUS, OHIO, A CORPORATION OF DELAWARE.

## MOTOR FUEL.

No Drawing.

Application filed March 7, 1928. Serial No. 259,926.

The present invention relates to liquid fuels for use in internal combustion engines, and more particularly to gasoline or other suitable petroleum distillates.

- 5 In the operation of an internal combustion engine, owing to the combustion of the fuel in the cylinders and the exceedingly high temperatures resulting therefrom, there is a more or less rapid accumulation of deposit in 10 the combustion chambers of the cylinders around the valves and upon the spark plugs, and also on the heads of the pistons, which seriously interferes with the proper operation of the engine. This deposit, commonly referred to as "carbon", tends to cause pre- 15 ignition of the fuel charge in the cylinders, resulting in what is commonly called a carbon "knock". The "carbon" deposit is not entirely carbon but includes other foreign 20 substances, such as iron, rust, or other metallic particles from the walls of the cylinders and the pistons, and generally a considerable portion of mineral matter due to the dust from the road being drawn into the cylinders 25 with the air entering the carburetor of the engine. The carbon element of the deposit is formed by soot resulting from incomplete combustion of the fuel and also from a carbonization of the excess of lubricating oil 30 which finds its way into the combustion chambers of the cylinders. In some instances this deposit is hard and dry, and in other instances it is more or less soft or sooty, and frequently it is greasy. This latter condition is very 35 objectionable because it tends particularly to foul the spark plugs and prevent proper ignition. The lubricant which finds its way into the combustion chambers does not perform its proper function in the said combustion chambers, because of the high temperatures prevailing in the latter. It is easily understood, however, that these chambers should receive proper lubrication.

- The main object of the present invention 45 is to provide a motor fuel comprising gasoline, or other suitable petroleum distillate, and certain ingredients in solution therein, which not only has the effect of preventing deposition of carbon upon the working parts 50 of internal combustion engines, but also tends to loosen and remove that which is present; and which not only improves the lubrication in the combustion chamber, where the lubrication is very often insufficient, but also possesses a higher gravity and generally pro-

vides considerably more power than those now commonly in use.

The ingredients employed are gasoline or other products of petroleum distillation, a high test lubricating oil, castor oil, paranitrochlorobenzene and benzol. The proportions of these ingredients may be varied, but a highly satisfactory and efficient liquid fuel has been obtained by the use of the said ingredients in the following proportions, to- 60 65

|                        |     |           |
|------------------------|-----|-----------|
| Gasolene               | 500 | gallons.  |
| Lubricating oil        | 34  | fluid oz. |
| Castor oil             | 17  | fluid oz. |
| Paranitrochlorobenzene | 12  | oz.       |
| Benzol                 | 65  | fluid oz. |

The lubricating oil and the castor oil are mixed together, paranitrochlorobenzene is dissolved in the benzol, and the solution so obtained added to the mixture of lubricating oil and castor oil. After suitably mixing and blending these materials, the compound so obtained is added to the gasoline or other product of petroleum distillation, whereby 75 the improved fuel is ready for use. This fuel is used in the ordinary manner, although in some cases it is necessary to adjust the carburetor on the engine differently than when used with gasoline alone. 80 85

The compound added to the gasoline is readily soluble therein or in other petroleum fuels used, and does in no way interfere with the explosion of the combustible charges in the cylinders. On the contrary, it tends to 90 improve the burning of the charge. Inasmuch as the compound is entirely and readily soluble in petroleum fuels, it is readily carburetable therewith. The primarily solvent part of the compound is the paranitrochlorobenzene, which is a coal tar product. This ingredient has a much higher boiling point than gasoline and is adapted to be absorbed by the carbon deposits and to have a solvent action upon those ingredients of the deposits which 95 are capable of being dissolved. The benzol not only serves as a solvent for the paranitrochlorobenzene, but acts also as a solvent for the carbon deposits. The mixture of lubricating oil and castor oil has a high heat test, 100 is not affected by the explosion of the successive charges in the cylinders of the engine, that is to say ignition does not injure it in its capacity as a lubricant to any considerable extent, and consequently the lubricant per- 105 110

forms its lubricating function in the combustion chambers of the engine. Furthermore, it also prevents carbon from adhering to the walls of the cylinders, spark plugs, 5 valves, cylinder rings, valve seats, etc., so that these elements are at all times kept clean, which is not the case when it is attempted to introduce ordinary lubricants with the fuel.

It has also been found that the compound 10 added to the gasolene acts as a catalytic agent and that, as a result of such action, the formation of carbon and its deposition upon the working parts of the engine are prevented. The compound added to the gasolene raises 15 the gravity of the fuel, assures material saving in gasolene together with a quick pick-up in the engine, and makes it possible to obtain materially increased power, as actual tests have shown. The new fuel composition 20 is adapted for use and with materially improved results in the same automobile engines now in use with gasolene, and without requiring any changes in the design of the engines. It also materially increases the flexibility 25 in speed of an internal combustion engine. It is a well known fact that the increased flexibility in speed is one of the principal reasons given by manufacturers for complicating the engines of automobiles by 30 increasing the number of the cylinders, so that the increased flexibility and speed obtainable with the improved fuel composition

makes it possible to obtain with a lesser number of engine cylinders a flexibility such as it has heretofore been considered necessary 35 to obtain by an increased number of cylinders.

What I claim is:—

1. A fuel composition for internal combustion engines consisting of hydrocarbon motor fuel material, a lubricant comprising a high heat test lubricating oil and castor oil, and a coal tar product comprising benzol and para-nitrochlorobenzene. 40

2. A fuel composition for internal combustion engines consisting of hydrocarbon motor fuel material, a lubricant comprising a high heat test lubricating oil and castor oil, and a coal tar product comprising benzol and para-nitrochlorobenzene, the para-nitrochlorobenzene being present in the proportion of 12 oz. 45 50 to 500 gallons of the fuel.

3. A fuel composition for internal combustion engines consisting of a hydrocarbon motor fuel material, a lubricant having a high boiling point, and a coal tar product comprising benzol and para-nitrochlorobenzene. 55

4. A fuel composition for internal combustion engines including a hydrocarbon motor fuel material, and a coal tar product comprising benzol and para-nitrochlorobenzene. 60

Signed at Columbus, in the county of Franklin and State of Ohio, this 7th day of February, A. D. 1928.

EARL C. HENNEN.